

Sept. 11, 1934.

E. L. DAVENPORT

1,973,431

## METHOD AND APPARATUS FOR COATING METAL STRIP

Filed Dec. 7, 1932

2 Sheets-Sheet 1



INVENTOR

Byrnes, Stebbins, Parmelee & Blenko

Sept. 11, 1934.

E. L. DAVENPORT

1,973,431

METHOD AND APPARATUS FOR COATING METAL STRIP

Filed Dec. 7, 1932

2 Sheets-Sheet 2

Fig. 2.



INVENTOR  
Edward L. Davenport  
by his attorneys  
Byrnes, Stebbins,  
Parmelee & Blenko

## UNITED STATES PATENT OFFICE

1,973,431

METHOD AND APPARATUS FOR COATING  
METAL STRIPEdward L. Davenport, New Castle, Pa., assignor to  
Johnson Bronze Company, New Castle, Pa., a  
corporation of Pennsylvania

Application December 7, 1932, Serial No. 646,135

7 Claims. (Cl. 207—11)

My invention relates to a method and apparatus for coating and, in particular, to the coating of metal strip. The specific application of the invention which I now contemplate is the 5 coating of steel strip with non-ferrous metal having a high fusing temperature, such as bronze or brass, for the purpose of making steel backing bearings with linings of suitable bearing metal.

10 It is known that in the welding or brazing of brass or bronze to steel, it is necessary to use fairly high temperatures, in the neighborhood of 2000° F. This temperature must be maintained at the point of application of the bronze 15 to the steel so that the molten bronze will penetrate the surface pores of the steel to form an intimate union therewith. This condition has heretofore not been obtained, so far as I am aware, in a continuous coating process or 20 apparatus.

I have invented a method and apparatus capable of satisfactorily providing a continuous steel strip with a coating of bronze or other bearing metal of suitable thickness to form a bearing 25 bushing. In accordance with my invention, I provide a source of molten bronze adjacent a continuously moving steel strip. I provide means for heating the strip as it moves past 30 the source of molten metal, and means for conducting a continuous stream of the latter to the strip. In order to prevent oxidation of 35 the steel strip, I enclose it in a chamber having a non-oxidizing atmosphere. I thus prevent the formation of an oxide layer on the steel which would prevent perfect adherence of the bronze 40 layer applied thereto.

For a complete understanding of the invention, reference is made to the accompanying drawings illustrating present preferred embodiments thereof.

In the drawings—

Figure 1 is a sectional view which is largely diagrammatic, illustrating one form of apparatus for carrying out the method of my invention;

Figure 2 is a partial view showing a portion of the apparatus of Figure 1 to enlarged scale;

Figure 3 is a sectional view taken along the line III—III of Figure 2; and

Figure 4 is a view similar to Figure 1, showing a modified form of apparatus.

Referring now in detail to the drawings, I provide a housing 10 lagged with any suitable insulating material. At one end of the housing 55 10, pinch rolls 11 are mounted in any suitable

bearings. Driving means of any convenient character (not shown) are provided for the pinch rolls 11. The rolls make a substantially gas-tight joint with the walls of the housing. Idler pinch rolls 12 are similarly mounted at 60 the other end of the housing 10 which is the entrance end. The pinch rolls 11 and 12 provide means for drawing a length of steel strip 13 through the housing 10. Within the housing 14 is provided for directing and supporting the strip.

A supply pipe 15 connects with the housing 10 to admit inert gas or other non-oxidizing or deoxidizing atmosphere to the housing 10. Preferably, the gas in the housing is maintained under a pressure slightly above that of atmosphere, and any leakage between the housing and pinch rolls is immediately made up by additional gas supplied through the pipe 15.

A bronze pot 16 mounted above the housing 10 provides a source of molten metal for application to the continuously moving strip 13. Preferably, the bronze is melted in any suitable type of furnace and poured into the pot 16. Heating means should be provided for the pot 16 to make up radiation and other losses, but the nature of such means is not material to the present invention. As an example thereof, I have shown a high frequency induction coil 17 which operates 80 in a well-known manner to produce eddy currents in the molten mass of metal which maintain the mass at the desired degree of temperature.

Extending downwardly from the pot 16 and 90 through the housing 10 is a spout 18 having a passage 19 therethrough of the cross-sectional shape illustrated in Figure 3. The spout is preferably of refractory non-conducting material and extends downwardly through the housing 10 to a point close to the guide 14 as shown in Figure 2.

In addition to maintaining the mass of metal in the pot 16 at the proper temperature, it is 100 also important to maintain that portion of the metal flowing through the passage 19 at a temperature such that it will bond properly with the steel strip 13 as it flows thereupon. For this purpose, I provide a generator 20 connected through a no-voltage relay 21 and a sliding contact of any suitable construction to the pinch rolls 12. The no-voltage relay 21 is of standard construction and is employed to open the generator circuit upon failure of the voltage therein 105 to prevent shunting of other circuits to be de-

scribed later. The generator 20 is also connected to a terminal 22 extending into the molten metal in the pot 16. A circuit is completed through the molten metal in the pot and that in 5 the passage 19 and the strip 13 between the spout 18 and the pinch rolls 12, so that current flows through said circuit. The effect of this current is first to preheat the strip 13 as it passes through the housing 10; second, the current also 10 has the effect of heating the metal in the passage 19 of the spout 18. The increased resistance of that portion of the circuit leads to the generation of a major portion of the heat therein, so that the molten metal as it flows through 15 the spout onto the strip 13 is heated to the proper degree which, of course, is susceptible of easy control by varying the current supply of the generator 20.

The guide 14 supports and directs the strip 13 as it moves through the housing 10 and under the spout 18. With the conditions as described, 20 of course, the strip 13 is preheated in traveling from the pinch rolls 12 to the spout 18 where it receives its layer of molten bronze indicated in 25 Figure 2 at 23. Both the steel strip 13 and the bronze coating 23 are prevented from oxidation by the deoxidizing or non-oxidizing atmosphere supplied through the pipe 15. After the strip has passed beneath the spout 18, it is further 30 heated to maintain the bronze layer molten for a sufficient length of time to permit proper alloying thereof with the steel base. This heating is accomplished by a generator 24 connected through a no-voltage relay 25 and a sliding contact to the pinch rolls 11. The generator 24 is 35 also connected to the pinch rolls 12. Heating current is thereby supplied to the full length of the strip 13 between the pinch rolls 11 and 12 and to both the coated and uncoated portions 40 thereof. The generator 24 also aids in the pre-heating of the strip 13, as well as maintaining the bronze layer at the proper temperature for the required interval.

The pinch rolls 11 and 12 are preferably 45 water-cooled, as indicated, by any convenient means to prevent their attaining excessive temperatures. The rolls 11, furthermore, exert a cooling effect on the coated strip so that the bronze layer applied thereto hardens and forms 50 a permanent bond with the steel base.

Referring now to Figure 4, I have illustrated a modified form of apparatus for carrying out the method, which is similar in some respects to the apparatus shown in Figure 1. Corresponding 55 elements are indicated by the same reference numerals. The features of the apparatus of Figure 4 differing from those of Figure 1 are the means for preheating the steel strip indicated at 13, and the means for maintaining 60 fluid the molten metal in the discharge spout of the pot 16.

As shown in Figure 4, a conduction heater 26 is disposed within the housing 10 and is connected to any suitable source of current. The 65 strip 13 passes through the heater 26 and its temperature is thereby raised to the proper point for the application of a layer of molten bronze.

The bronze pot 16 in Figure 4 has a discharge spout 27 with a central passage 28 therethrough 70 of cross section similar to the passage 19 of Figure 1. For maintaining the fluidity of molten bronze passing through the spout 27 and for further heating the strip 13, I provide a high frequency induction coil 29 having portions disposed above and below the spout and 75

strip. The effect of such coil, of course, is to induce eddy currents in the bronze in the passage 28 and the strip 13, which heat the metal to the desired degree. The guide 14 may be of a high temperature alloy metal so that it also is 80 heated by the induced currents.

The operation of the apparatus shown in Figure 4 is substantially the same as that of Figure 1. The strip 13 is drawn through the 85 housing 10 by means of the driven pinch rolls 11, is preheated by the heater 26, and is then given a layer of molten bronze delivered through the spout 27. The bronze layer as it is delivered and the strip 13 as it approaches the spout 27 90 are heated by induction to the proper point. The proper brazing temperature for bronze is about 2200° F., and if the steel strip is heated to this temperature or slightly therebelow, a 95 satisfactory alloying or welding of the bronze to the steel will occur.

It will be apparent from the foregoing description that the invention provides highly useful means for applying a coating of bearing metal to a continuous steel strip at a high rate and 100 at very low cost. The base or backing strip can be obtained in long lengths so that the operation of the coating apparatus can be made fairly continuous. By maintaining the molten metal at the proper brazing temperature at the 105 point where it engages the backing strip, a satisfactory union therebetween is assured. The flow of molten bronze from the bronze pot may, of course, be controlled by any suitable means not shown. In case of failure of the voltage 110 in any of the heating circuits of Figure 1, the no-voltage relays immediately operate to open the circuits and prevent shunting of the other circuits in parallel therewith. The preheating of the steel strip prevents the possibility of chilling the bronze upon contact with the strip, which would otherwise occur. Since the pre-heated strip is maintained in a non-oxidizing atmosphere, the formation of any oxide coating 115 thereon is precluded. This preserves the initial 120 clean surface of the strip for receiving the bronze layer. The invention, of course, is useful in connection with the application of a coating of metals other than bronze or brass to a backing strip, whether of steel or some other material. 125

Although I have illustrated and described but two preferred embodiments of the invention, it is obvious that numerous changes therein may be made without departing either from the spirit 130 of the invention or the scope of the appended claims.

I claim:

1. In a method of coating strip, the steps including subjecting a continuous strip to a pre-heating operation, supplying a non-oxidizing atmosphere in the vicinity of the preheated strip, delivering a stream of liquid coating material onto one side of the strip, maintaining the other side of the strip substantially free from contact with said stream, and further heating the strip and coating after application of the latter to the strip.

2. Apparatus for coating strip comprising strip-feeding means, means for delivering a stream of molten coating material to one side of a moving strip actuated by the feeding means, means for heating the strip prior to receiving the coating material, means for supporting the strip at the point of delivery of said 145

- stream, and means for heating said stream at said point of delivery. 5. In a coating apparatus, strip feeding means, a container for coating material having a spout communicating with the strip, and means for supplying electric current to the material in the container and spout and to said strip for heating purposes. 80
3. In a coating apparatus, strip feeding means, a guide for supporting the strip as it is being fed, a source of coating material above the strip, a spout from said source extending to a point over said guide, and means for electrically heating said strip, the coating material in said spout and the source of coating material, including a contact projecting into the latter. 6. In a coating apparatus, strip feeding means, a container for coating material, a spout extending from the container for delivering material onto the strip, and means for inductively heating the spout and the strip adjacent the point of delivery of the former. 85
4. In a coating apparatus, strip feeding means, a guide supporting the strip as it is being fed, a source of coating material adjacent thereto, and a spout extending from said source to a point above said guide, of means for supplying heating current to the strip approaching said guide, and means for electrically heating the coating material adjacent the point of delivery to the strip, including a contact projecting into said source. 7. Apparatus for coating a strip with a conducting material including a container for the material, strip advancing means, a passage for material to flow through from the container to the strip, and means for electrically heating the material, including a contact projecting into the container. 90

EDWARD L. DAVENPORT. 95

|    |  |     |
|----|--|-----|
| 25 |  | 100 |
| 30 |  | 105 |
| 35 |  | 110 |
| 40 |  | 115 |
| 45 |  | 120 |
| 50 |  | 125 |
| 55 |  | 130 |
| 60 |  | 135 |
| 65 |  | 140 |
| 70 |  |     |
| 75 |  |     |